

March 25, 1941.

F. E. DRUMMOND

2,236,397

METHOD OF DRYING FINISHES

Filed April 17, 1939

2 Sheets-Sheet 1

FIG. 1



FIG. 2



FIG. 3



FIG. 4



INVENTOR.

BY *Folsom E. Drummond*

ATTORNEYS

March 25, 1941.

F. E. DRUMMOND

2,236,397

METHOD OF DRYING FINISHES

Filed April 17, 1939

2 Sheets-Sheet 2

FIG. 5



FIG. 6



INVENTOR.

BY *Folsom E. Drummond*  
*Doulman & Doulman*  
ATTORNEYS

## UNITED STATES PATENT OFFICE

2,236,397

## METHOD OF DRYING FINISHES

Folsom E. Drummond, Dayton, Ohio, assignor, by  
mesne assignments, to New Wrinkle, Inc., Wil-  
mington, Del., a corporation of Delaware

Application April 17, 1939, Serial No. 268,217

6 Claims. (Cl. 34—24)

My invention relates to a method for drying coating compositions, and more particularly to the method of producing wrinkle finishes. The invention, however, is adapted for accelerating the drying of various types of coating compositions which dry to a hard flexible film by oxidation, polymerization, evaporation of solvents or a combination of these actions.

It is one object of this invention to produce wrinkle finishes comprising conventional non-wrinkling oil vehicles such as linseed, perilla, soya bean oil, poppy seed, fish oils and the like, which oils ordinarily dry to a smooth, glossy, non-wrinkling film.

Another object is to provide a method for producing articles having wrinkle finishes from compositions comprising blends of non-wrinkling and wrinkling oils, which wrinkling oils include China-wood, oiticica, and poyok in blown, unblown or raw state.

Another object is to provide an improved method of drying coated compositions of the drying oil or oleoresinous type which ordinarily dry to a smooth surface so that they will dry to a wrinkle finish.

Another object is to provide an improved method of accelerating the surface drying of coating compositions in order to produce a wrinkle or irregular surface film.

Another object of this invention is to provide a controllable atmosphere for baking coated articles to cause the coating to dry to a hard, smooth finish or irregular wrinkle surface as desired.

Another object is to provide an enclosure for force air drying coated articles by means of oxygen or ozone enriched heated air which also carries small amounts of an oxidation promoting catalyst for increasing the oxidation activity on the film surface so as to produce a wrinkle finish.

Another object is to provide an improved method of accelerating the oxidation and polymerization of coating compositions applied to articles in a thin film so as to lessen the time for drying coating films to a dust-free finish.

In general the wrinkling of coated films is brought about by unequal drying of the film producing surface volume changes which develop introverted folds in the surface skin of the film, producing a wrinkle finish. In the case of drying oil coating films comprising wrinkling oils, for example China-wood or oiticica, it has been found that folds or wrinkling of the film surface may be brought about by excess oxidation and

polymerization at the surface of the film. This invention provides an improved method of effecting this to produce a wrinkle coating on articles.

In the accompanying drawings:

Figure 1 is a vertical sectional view of an article having a smooth surface coating;

Figure 2 is a vertical sectional view through an oven showing the manner of exposing the material to heat and ultra-violet ray lamps for 10 drying coated articles;

Figure 3 is a similar sectional view illustrating the arrangement for baking finishes which are applied to both sides of panels or sheets;

Figure 4 is a similar view in section taken 15 through a circular oven having heat and ultra-violet ray lamps mounted around the interior wall to concentrate the heat and light on irregular shaped articles which are to be dried to a wrinkle finish;

Figure 5 is a similar view of an oven as in Figure 1, illustrating the utilization of heat lamps alone with means for admitting oxygen to enrich the atmosphere in contact with the coated article;

Figure 6 is an elevation view, partly in section, of an oven showing the arrangement for admitting heated air which has been enriched with oxygen and having an oxidation catalyst incorporated therewith for drying coated articles to produce a wrinkle finish.

Referring to the drawings in detail, Figure 1 shows a panel or article A having a smooth surface coating B. In Figures 2, 3 and 4 an oven generally designated 10 is illustrated for drying coated articles, according to my invention, to accelerate the drying of the coating to a hard smooth film or wrinkle surface finish.

The ovens are constructed in the form of tunnels or rectangular enclosures having suitable 40 means for supporting and conveying coated articles into and out of the drying oven. Heat is supplied by banks of reflector equipped incandescent lamps 11 which are arranged within the enclosure so as to concentrate the rays onto 45 the surface of the coated articles. Preferably infra-red radiating electric lamps having carbon filaments are used for this purpose.

Interposed between the heat lamps 11 are ultra-violet irradiating means 12. Any suitable 50 source of ultra-violet ray producing means can be employed, the quartz mercury arc lamp of the Cooper-Hewitt type being readily applicable. Ultra-violet irradiation from a carbon arc may also be used if desired. The heat lamps and 55

ultra-violet lamps may be arranged in alternate relationship so as to provide even distribution of heat and ultra-violet irradiation of the atmosphere adjacent the articles being dried. In general the lamps should be placed between ten and thirty inches from the coated article. The light drying enclosures are not hermetically sealed so as to permit the ready exit of products of oxidation during drying of the coated articles.

In the modification illustrated in Figure 4 the oven 13 is of circular construction and the heat and ultra-violet lamps are maintained in spaced relationship around the walls so as to effectively direct the rays against all sides of an irregular shaped article. The lamps may, if desired, be made adjustable so that their position can be changed relative to each other. It will also be understood that the number of heat lamps or ultra-violet lamps may be varied as required to increase or decrease the temperature of the enclosure and the ultra-violet irradiation of the atmosphere.

Ultra-violet irradiation provides means for ionizing the air in contact with the coating film forming ozone which accelerates the surface drying by auto-oxidation. This oxidation of the coating is enhanced by the heat lamps resulting in rapid surface drying of the film which expands laterally due to the oxidation and increased volume to produce folds or creases over the entire film surface. By this method of accelerating the surface drying rate of films, coating compositions particularly of the drying oil type, which under the ordinary drying and baking temperatures do not produce a wrinkle finish, are made to dry to a satisfactory wrinkle finish. Heretofore in the compounding of wrinkle finishes, the use of substantial amounts of tung oil, oiticica oil or synthetic wrinkle resins of the drying oil acid modified type has been required for the production of wrinkle finish coating compositions. By the improved method of accelerating the surface drying rate of coating compositions according to this invention, the use of large amounts of these expensive drying oils is unnecessary and in general may be substituted by linseed oil, soya bean oil and the like non-wrinkling oils.

In Figure 5 the baking oven 14 comprises an endless conveyor 15 which is arranged for conveniently moving the coated articles into and out of the light drying enclosure. In this instance ultra-violet lamps are omitted and the heat lamps 11 alone used. Oxygen or ozone enriched air is introduced into the drying oven as at 16. Where drying oil compositions used in coating the articles comprise raw China wood oil or similar drying oils which have not been heat treated to a sufficiently high temperature to eliminate crystallization or gas checking, the nitrogen dioxide content of the atmosphere may be maintained above 4 to 5 parts per million parts of air which brings about crystallization or gas checking of the film. Ordinarily, however, gas checking will not be produced even with articles coated with raw drying oils due to the comparatively short period of time between the evaporation of the solvents and the beginning of oxidation.

The usual drying oil coating compositions comprise metallic oxidation catalysts such as cobalt, manganese, lead in the form of linoleate or acetate, alone or mixtures of these. These driers enhance the wrinkling and materially speed up the drying of the film especially when dried by the use of heat lamps as in this invention. To

accentuate surface oxidation atomized organic solutions of metallic driers such as cobalt or manganese in the form of oleates, stearates, naphthenates, etc. may be introduced into the drying ovens to form a part of the atmosphere in contact with the coating film. Metal driers colloidally dispersed in an oil soluble solvent such as butyl alcohol or petroleum spirits may be utilized.

This modification is illustrated in Figure 6 wherein the required temperature in the oven 17 for baking the coated articles is maintained by the introduction of preheated air, as shown, into which has been introduced oxygen or ozone enriched air together with an oxidation catalyst. It will be understood that heat lamps may be employed together with the circulating heated air for maintaining the temperature in the baking oven 17 if desired. A fan generally designated 18 may be employed for forcing the circulation of air through the heating element 19 and circulating it through the oven, as shown in Figure 6.

The oxidation catalyst which may be introduced into the oven may comprise atomized organic peroxide such as acetyl or phthalyl or benzoyl peroxide dissolved in benzol or toluol. This solution may be suitably sprayed into the oven chamber or carried into the oven by the oxygen or stream of air being conducted into the oven. In this manner sufficient amount of oxidation catalyst can be placed in contact with the surface of the coating film on the articles to accelerate the surface oxidation and drying of the coating to produce a satisfactory wrinkle finish. This will be enhanced further by the use of coating compositions comprising metallic driers. Clear varnishes as well as pigmented enamels may be dried to a wrinkle finish.

The usual temperatures employed in producing wrinkle finishes on metal surfaces are of the order of 150 up to approximately 450 degrees F. For producing wrinkle finishes on wood, paper and similar materials somewhat lower temperatures, such as 120 to 150 degrees F. may be used. The elevated temperatures produce a more rapid oxidation of the film surface and promote the production of wrinkle finishes and in general accentuate the wrinkle. Lower temperatures of baking usually require higher percentages of drying oils having poly-conjugated double bond structure in order to sufficiently accelerate the oxidation rate of the film surface during the treatment to produce a wrinkle or irregular surface finish.

As an alternative manner of contacting the surface of the coating film with the oxidation catalyst, a thin film of the solution carrying the catalyst may be lightly sprayed over the coating just prior to introducing the coated articles into the baking oven. Further in place of the oxidation catalyst mentioned, oxidized turpentine which is high in active peroxide of oxygen may be utilized with or without the addition of metallic drier.

It will be understood that I desire to comprehend within my invention such modifications as come within the scope of the claims and the invention.

Having thus fully described my invention, what I claim as new and desire to secure by Letters Patent is:

1. The method of producing a wrinkle finish comprising drying oxidizable coating compositions in the form of a film including the steps of heating air, introducing oxygen in said air to increase the oxygen content above that normally

present in ordinary air, admixing an oxidation catalyst into said air and subjecting the coating film to said air into which the oxygen and catalyst have been introduced.

5. 2. The method of producing wrinkle finishes comprising drying oxidizable compositions in the form of a film comprising the steps of concentrating infra-red heat rays onto said film, heating air and simultaneously introducing oxygen 5 thereinto to increase the oxygen content above that normally present in ordinary air, and subjecting the coating film to said air into which oxygen has been introduced to effect drying of the coating to a wrinkled surface.

10. 3. The method of producing wrinkle finishes from oxidizable paints, varnishes, and resinous compositions which comprises the steps of focusing heat rays on to the film surface, heating air, incorporating oxygen in said air to increase the 15 oxygen content above that normally present in air, concurrently adding oxidation catalyst into said heated air and subjecting the coated articles thereto to produce a wrinkled surface coating.

15. 4. The method of producing a wrinkle finish 20 from coating compositions comprising non-wrinkling oils consisting of drying the coating in the form of a film and accelerating the surface drying of the film by heating the air in which the

coating film is to be dried, introducing oxygen into said air to increase the oxygen content of the heated air above that normally present in ordinary air, and spraying the coating film with an oxidation catalyst immediately prior to drying said film to effect accelerated oxidation and drying of the film at its surface whereby an irregular wrinkled surface is produced. 5

5. The method of producing a wrinkle finish by treating an article having a film of the coating 10 composition thereon, comprising spraying a light coating of a solution containing an oxidation catalyst over said coating film just prior to drying said coating film, subjecting the film to heated air, introducing oxygen into said air and drying 15 the coating film in said heated air to produce folds or creases in the surface of the film and form an irregular wrinkled finish.

6. A method of producing a wrinkle finish by accelerating the surface drying of the composition 20 in the form of a film comprising the steps of concentrating infra red heat rays onto the surface of the film and simultaneously subjecting said film to air in which oxygen content has been substantially increased above that normally 25 a constituent part of air.

FOLSOM E. DRUMMOND.